

(No Model.)

E. P. CLARK.  
ELECTRODEPOSITION OF LEAD.

No. 598,313.

Patented Feb. 1, 1898.



WITNESSES:

Fairh. S. Ober.  
Harry Bailey.

INVENTOR

Ernest P. Clark  
BY  
M. M. Rosenthal  
ATTORNEY

# UNITED STATES PATENT OFFICE.

ERNEST P. CLARK, OF NEW YORK, N. Y., ASSIGNOR OF ONE-HALF TO  
CHARLES S. CAMPBELL, OF SAME PLACE.

## ELECTRODEPOSITION OF LEAD.

SPECIFICATION forming part of Letters Patent No. 598,313, dated February 1, 1898.

Application filed June 8, 1897. Serial No. 639,908. (Specimens.)

*To all whom it may concern:*

Be it known that I, ERNEST P. CLARK, a citizen of the United States, residing at New York, in the county of New York and State 5 of New York, have invented certain new and useful Improvements in Electrodeposition of Lead, of which the following is a full, clear, and exact description.

This invention relates to the production of 10 a peculiar form of finely-divided metallic lead by means of electrodeposition; and it consists of certain novel means and methods of preparing a bath or solution from which a form of finely-divided lead heretofore unknown is produced by electrolysis, to which 15 form I have given the title of "feathery" lead, on account of its peculiar appearance in the depositing solution.

The accompanying drawing shows a 20 sectional view of an electrodepositing cell equipped for operation in accordance with my invention.

If a solution be made of dilute acetic acid, 25 nitric acid, acetate of lead, or of any of the well-known solvents of lead and an anode of metallic lead be immersed in the said solution, a cathode of lead or other suitable material being also placed in the solution, and an electric current be sent through the bath 30 or solution, a deposit of slate-colored lead without metallic luster and devoid of metallic appearance or tenacity is produced upon the cathode. This deposit has been aptly 35 termed "frothy" lead, and, to my knowledge, is the only form in which lead in or approaching the metallic state has been deposited by the aid of electricity.

The lead produced by precipitating the 40 metal from its acetic solution by means of metallic zinc is another variety of finely-divided lead and is known as "spongy" lead. This variety has more of a metallic appearance than the frothy lead and may be compressed into somewhat solid and firm masses 45 or blocks, but is not a bright and lustrous material, nor has it the tenacity of the material formed by my process, which I will now proceed to describe.

In preparing my solution I take water and 50 acetate of lead—about one pound ten ounces of acetate of lead to each gallon of water. A

slightly-different proportion may be used, according to the purity of the acetate. About half of the above amount of the acetate can be readily and quickly dissolved in the water 55 by stirring. The balance should be placed in a coarse cotton bag and suspended in the solution near its surface. Now a piece or pieces of clean metallic zinc are placed in the solution, preferably in a vertical position, 60 and left for about twelve hours. By the chemical action now taking place the lead contained in the solution is precipitated upon the zinc and a portion of the zinc is dissolved, replacing the lead in the solution. At the 65 same time as lead is being removed the solution will rapidly dissolve the portion of acetate of lead contained in the cotton bag, the solution thus growing more dense or of greater specific gravity. After about ten or 70 twelve hours all the acetate has been dissolved from the bag, which can then be removed. The zinc plates should also be removed and the heavy deposit of spongy lead detached. Upon replacing the zinc plates a 75 new deposit of spongy lead will rapidly form.

As lead is removed from the solution and zinc dissolved therein the specific gravity of the solution will become gradually less. This process, which is a change from acetate of 80 lead to acetate of zinc, should be stopped by removing the zinc plates before all the lead is removed from the solution.

I have found in practice that in using the 85 above proportions of acetate and water the zinc should be removed and the process of conversion stopped when the gravity of the solution is reduced to 18° or 19° of Baumé's hydrometer. The solution will now be of a light-brown color, or if sulfate of lead is contained as an impurity in the acetate there 90 may be a milky turbidness also present which will subside in a few hours and do no harm. If now a lead anode and a cathode of lead or other suitable material be immersed in the 95 liquid and a current of electricity be sent through it, there will usually appear in a few minutes bright deposits of metallic lead upon the cathode and no trace of the slate-colored frothy lead mentioned above. Sometimes, 100 however, the first deposit which appears is the frothy material, and at other times both

kinds of deposit appear. The anode and cathode should be first placed vertically until it is certain that the frothy deposit is not being formed, after which the disposition about 5 to be described may be adopted.

I find in practice that the frothy form of deposit is rarely seen in this solution unless its specific gravity is too low. The gravity I have mentioned is that which I have found 10 best adapted to the purpose, but it may be much lower, if desired, and good results obtained. One way I have found for obtaining a good working solution of a low gravity is to use about half the amount of acetate of lead 15 above mentioned and then remove nearly all of the lead from the solution by means of zinc, as described. The vertically-arranged anode and cathode being now placed in the solution and the current passed, the anode is 20 gradually dissolved and a diffused deposit of the frothy form appears and must be removed from the cathode from time to time. After a time, varying from one or two to forty-eight or more hours, a bright deposit will be observed 25 on the lower part of the cathode, which is the desired deposit of "feathery" lead. Continuing the current and removing the deposit from time to time there will gradually be more of the feathery bright deposit and less of the dull 30 slate-colored deposit, until finally the whole of the lead deposited will be bright, silvery, and feathery in appearance. A little pulverized acetate of lead—say an ounce to the gallon—added to the solution after the bright 35 deposit first appears will hasten the process. By this means a solution as light as 8° or 10° Baumé can be obtained which will work perfectly; but I prefer to use it of a higher density, as first described, as being easier to 40 form and of lower electrical resistance.

The solution being formed in either of the above ways I place it in a large glass jar or tank *a*, holding several gallons. A cathode *b*, consisting of a disk of thin sheet-lead, is 45 placed in the bottom of the tank, with an insulated conductor *b'*, extending above the liquid, soldered to the disk. A heavy anode *c*, of cast or pig lead, is suspended in the solution near its surface and the current passed. 50 The anode gradually dissolves and very soon a deposit of lead of the general form of very small feathers is seen to grow upon the cathode and gradually increases in heaps or piles, starting at the edges of the cathode and gradually covering all its surface, filling the jar 55 several inches. During the first few hours the solution gradually loses its brown tinge and becomes perfectly clear. The deposit becomes of a silvery brightness and the re- 60 semblance of the crystals to small feathers becomes very striking. The deposit should be gently pushed down with a wooden rod from time to time until sufficient of the material has been made. The density of the 65 current to be used cannot be definitely stated, as I have found that good results have been obtained with a current ranging anywhere

from one to sixteen amperes per square foot of anode. If a portion of this material be removed and examined, it will be found to be 70 interlaced like felt or oakum, and in pulling it apart its tenacity is quite remarkable, being very much greater than that of spongy lead deposited from acetate-of-lead solution. If compressed in the hand or by other means, 75 it forms a strong tough mass, and when fresh is very bright and silvery in appearance, but of course soon turns dull from exposure to the air. This product in fact seems essentially to be a fibrous material free from all oxides 80 and other impurities.

As far as I understand the chemistry of the solution it consists of a mixture of acetate of lead and acetate of zinc, yet I have failed to obtain any such results from an ordinary mixture of these solutions. I have also tried unsuccessfully to use a solution of acetic acid by dissolving zinc in it electrolytically and adding lead by the same process. The only way I have found to produce this peculiar 90 form of deposited lead is by the solution produced as above described. I have also thought that as the solution contains a large amount of zinc some zinc may be deposited with the lead, but so far I have been unable to find 95 any trace of it in the material deposited. I believe this material will be largely used for the active material of storage-battery plates, for which purpose it possesses many advantages. I do not limit myself, however, to this 100 or any other particular use or application of my new material, but claim its use for all purposes wherein lead in an extreme state of subdivision may be employed and where a finely-divided lead of lustrous surface and feathery 105 or fibrous nature is desirable.

Having thus described my invention, I claim—

1. The process of producing finely-divided lead which consists in first partially changing 110 an acetate-of-lead solution into an acetate-of-zinc solution and then depositing lead by passing a current of electricity from a lead anode through the solution to a cathode, substantially as described.

2. The process of producing finely-divided lead, which consists in first putting zinc into a solution of acetate of lead and allowing it to remain until a portion of the lead in the solution has been deposited and zinc gone into 120 solution, and then passing a current of electricity from a lead anode through the solution to deposit the finely-divided lead upon the cathode, substantially as described.

3. The process of producing finely-divided 125 lead of a feathery and fibrous nature which consists in first dissolving acetate of lead in water, then immersing in this solution a plate of zinc and allowing it to remain until a portion of the lead has been deposited and a portion of the zinc substituted therefor in the solution; then passing a current of electricity through the solution from a lead anode to a cathode until the deposit of lead on the cath-

ode changes from a frothy appearance to a feathery appearance and then continuing the electrodeposition of the lead upon the cathode horizontally arranged in the lower portion 5 of the solution, substantially as described.

4. The process of electrodepositing lead, consisting in first displacing a portion of the lead in a lead acetate solution and substituting therefor some other material, and then

passing a current of electricity through the 10 solution from a lead anode.

In testimony whereof I subscribe my signature in presence of two witnesses.

ERNEST P. CLARK.

Witnesses:

FRANK S. OBER,  
HARRY BAILEY.